

# United States Patent

Panzer

[15] 3,664,955

[45] May 23, 1972

[54] **LUBRICATING OIL COMPOSITIONS OF IMPROVED THERMAL STABILITY**

[72] Inventor: Jerome Panzer, Roselle Park, N.J.

[73] Assignee: Esso Research and Engineering Company

[22] Filed: Dec. 31, 1969

[21] Appl. No.: 889,745

[52] U.S. Cl.....252/47.5, 252/45

[51] Int. Cl.....C10m 1/38

[58] Field of Search.....252/45, 47.5, 51.5 A

[56] **References Cited**

UNITED STATES PATENTS

|           |         |                    |            |
|-----------|---------|--------------------|------------|
| 2,312,750 | 3/1943  | Cohen.....         | 252/45 X   |
| 2,337,473 | 12/1943 | Knowles et al..... | 252/45 X   |
| 3,172,892 | 3/1965  | Le Suer et al..... | 252/51.5 A |
| 3,309,316 | 3/1967  | McNinch.....       | 252/47.5   |
| 3,352,782 | 11/1967 | Brasch.....        | 252/47.5   |
| 3,498,915 | 3/1970  | Coleman.....       | 252/45 X   |

Primary Examiner—Daniel E. Wyman

Assistant Examiner—W. Cannon

Attorney—Pearlman and Stahl and Ernest V. Haines

[57]

## ABSTRACT

Mineral lubricating oil compositions are prepared containing oil-soluble additives for sludge control, having improved high temperature oxidation stability and thus permitting longer periods of service before it becomes necessary to drain the used oil and replace it with fresh oil. The novel additive mixture is prepared by reacting elemental sulfur with long chain ( $C_{16+}$ ) oil-soluble olefinically unsaturated monomeric or polymeric hydrocarbons, e.g. polyisobutylene, and using such sulfurized compounds in conjunction with conventional ashless dispersants with or without using additional ashless dispersants which have previously been reacted with elemental sulfur. Many of the hydrocarbons used as starting materials, in their unsulfurized state, have heretofore been used as viscosity index improvers in lubricating oil compositions.

13 Claims, No Drawings

## LUBRICATING OIL COMPOSITIONS OF IMPROVED THERMAL STABILITY

## BACKGROUND OF THE INVENTION

The present invention relates to the use in mineral lubricating oil compositions of a combination of oil-soluble sulfurized olefinic compounds with the so-called ashless dispersants which are likewise oil-soluble and have been used in lubricating oil compositions for some years.

Numerous addition agents have heretofore been prepared for use in automotive mineral lubricating oils, including the so-called heavy duty oils which are also employed in railroad diesel engines and gas engines. The prior researchers have been successful in finding various types of oil-soluble organic compounds which exhibit specialized and specific properties of a beneficial nature when they are incorporated into these mineral lubricating oils. For many years now, organic compounds have been added in minor amounts to lubricating oils for the purpose of lowering their pour point, of improving their viscosity index, of affording increased resistance to oxidation, of imparting antiwear properties, of inhibiting sludge formation and of dispersing sludge when it is formed during use of the oils. The use of such additives at the present time enjoys widespread commercial acceptance. Good oxidation stability and good dispersing along with good detergency have become essential requirements for automotive lubricants. This is particularly so in connection with lubricating oils used in so-called heavy duty engines such as gas engines and railroad diesel engines. Additionally, the additives employed must necessarily be accepted from the standpoint of lack of wear or attack on the specialized types of bearings employed in internal combustion engines at the present time. Copper-lead-containing bearings are unusually susceptible to wear and corrosion problems. Suitable compounded oils must exhibit low corrosion and low bearing wear with respect to the specialized bearings which they contact in order to be acceptable commercially.

In the past, it has been proposed to add sulfurized polyisobutylene of relatively low molecular weight (boiling range 175°-260° C.) or of higher molecular weights, or derivatives thereof, to lubricating oils. See, for example, U.S. Pat. Nos. 2,279,688; 2,312,750; 2,330,858; 2,535,705 and 2,658,900. Also, it has been proposed in the past to employ sulfurized ashless dispersants in lubricating oils, see U.S. Pat. Nos. 3,390,086 and 3,309,316; whose disclosures are incorporated herein by reference. By the incorporation of elemental sulfur into a conventionally used olefinically unsaturated hydrocarbon, namely polyisobutylene, and by the incorporation of elemental sulfur into a conventional ashless dispersant, it was possible to increase the effectiveness of these materials for their intended purpose even in the case of lubricating oil compositions being subjected to extremely high temperatures during use. The thermal stability of the lubricating oils containing a combination of such additives, along with unsulfurized ashless dispersants, was greatly enhanced and resulted in the expended and more diversified, use of lubricating oils than when such oils contained either of these types of additives alone; because of the enhanced oxidation stability or resistance to oxidative degradation achieved by the introduction of the elemental sulfur into these compounds.

It has now been discovered that the use of sulfurized oil-soluble olefinically unsaturated long chain hydrocarbons in conjunction with a conventional ashless dispersant (with or without the use of a sulfurized ashless dispersant) gives rise to lubricating oils which have unusually high oxidation stability at high temperatures and which exhibit a heretofore unattainable degree of resistance to sludge formation and an excellent dispersion of the sludge that is formed. What this amounts to is that the versatility of lubricating oils as to their scope of use, where such oils contain this combination of additives, has been increased markedly because of the enhanced high temperature characteristics achieved by so compounding these oils. Another advantage lies in the fact that even when using

such compounded oils at lower temperatures or at temperatures ordinarily encountered in the automotive engines, the life of the oil is increased over that heretofore attainable and so such oils may be employed for longer periods of time necessitating fewer oil changes and longer engine running periods between changes. Whereas, heretofore, a heavy diesel engine operating under severe high temperature conditions would require an oil change after 1,500 hours of operation, because of oxidation breakdown of the oil and excessive sludge build-up due to high temperature conditions in the oil, it is now possible to increase the life of that same oil used under the same conditions by as much as 50 percent through the use of the combination of a sulfurized oil-soluble unsaturated hydrocarbon in combination with an ashless dispersant and, optionally, a sulfurized ashless dispersant.

The materials which may be treated with elemental sulfur or with sodium polysulfide, which is the chemical equivalent of elemental sulfur, are many and varied in number and constitute a great many of those oil-soluble unsaturated polymeric aliphatic hydrocarbon compounds possessing olefinic unsaturation which have heretofore customarily and conventionally been employed as viscosity index improvers in lubricating oils. It has now been discovered that the introduction into these olefinically unsaturated aliphatic hydrocarbon compounds, as well as into similar compounds not possessing V.I. improving properties, of elemental sulfur enhances their properties when used in lubricating oils. The ashless dispersants, used in combination, are well-known conventional and commercially available compounds. They may be employed in the form in which they are commercially available. They may be sulfurized, i.e. subjected to a reaction with elemental sulfur as described and claimed in the aforementioned U.S. Pat. No. 3,390,086 whose disclosure is incorporated hereinto by reference and used in conjunction with the conventional ashless dispersants of commerce.

Among the many varied types of olefinic unsaturated hydrocarbons which are used as starting compounds which are to be treated with elemental sulfur or its chemical equivalent such as sodium polysulfide are:

1. long chain (C<sub>16</sub>-C<sub>30</sub>) alpha monoolefin monomers or mixtures thereof;
2. homopolymers of C<sub>3</sub> to C<sub>18</sub> alpha monoolefins;
3. copolymers of C<sub>2</sub> to C<sub>18</sub> alpha monoolefins with different C<sub>3</sub> to C<sub>18</sub> alpha monoolefins; and
4. terpolymers of three different monomers of (3) or of two different monomers (3) with a diolefin such as methylene norbornene or butadiene or with still a third alpha monoolefin.

Exemplary of the reactants that may be employed as starting materials are the following: (copolymers are shown thus: monomer - monomer) C<sub>18</sub>+ alpha olefin mixtures, octadecene-1, hexadecene-1, tetradecene-1, C<sub>16</sub>-C<sub>18</sub> alpha olefins, polypropylene, polyisobutylene, ethylene-propylene, ethylene-isobutylene, ethylene-propylene-isobutylene, ethylene-propylene-butadiene-1,3, n-octene-1-isobutylene, propylene-pentene-2, ethylene-propylene-n-dodecene, ethylene-isobutylene-n-decene, ethylene-propylene-1,4-hexadiene, ethylene-propylene-dicyclopentadiene, ethylene-propylene-methylene norbornene. The number average molecular weights of the polymers, copolymers, or terpolymers generally range between about 300 and about 150,000, preferably between about 900 and about 70,000, and they are soluble in lubricating oils. These polymeric products are plastic solids, waxy or elastomeric depending on their molecular weights. Their physical properties and appearance are not the criteria that determine their efficacy, when sulfurized, and used in lubricating oils. The more highly amorphous (non-crystalline) products are preferred.

In general, crystalline contents of less than 25 wt. percent in the polymers are desirable and when such polymers are sulfurized, their use in lubricating oils affords viscosity index improving properties as well as oxidative and sludge inhibiting properties to the oils.

The polymerization reactions used to produce the polymeric hydrocarbon products are all well known to the art and the polymers are well-known commercial articles sold on the open market. The polymeric hydrocarbons are formed by polymerizing, copolymerizing, or terpolymerizing the olefinic monomers using Friedel-Crafts type catalysts, the so-called metallo alkyl, or coordination catalysts, or the Ziegler type catalysts. The homopolymers, i.e. polyisobutylene, most generally are produced by using Friedel-Crafts type catalysts such as boron trifluoride or aluminum chloride at low temperatures. Representative U.S. Pats. disclosing such products and their methods of preparation are Nos. 2,239,501; 2,534,095; 2,781,410; and 2,825,721 whose disclosures are incorporated herein by reference. The copolymers and terpolymers are usually produced by the use of coordination of metallo alkyl type catalysts. Representative U.S. Pats. disclosing suitable starting materials of these types, which may be sulfurized, are: Nos. 2,691,647; 2,975,159; 2,933,480; 3,051,690; and 3,389,087 whose disclosures are incorporated herein by reference. See also Canadian Patent No. 718,417 and French Pat. No. 1,537,571.

The ashless sludge dispersants are conventionally used in lubricating oils and are produced by condensing primary or secondary aliphatic amines, such as polyalkylene polyamines, with one or more long chain ( $C_{40}-C_{250}$ ) alkenyl substituted mono or dicarboxylic acids or anhydrides thereof. The alkenyl substituted dicarboxylic acid or anhydride is conventionally prepared and the final product, before condensation with the polyamine, has a number average molecular weight generally between about 700 and about 5,000, preferably between about 800 and about 2,000. Preferably, the alkenyl radical is derived from polyisobutylene or from a polypropylene. Alkenyl monocarboxylic acids for use in the present invention also will have molecular weights in the range of from about 700 to about 5,000, preferably between about 800 and about 2,000. The methods of preparation of the dicarboxylic acid materials are disclosed in U.S. Pat. No. 3,172,892, which disclosures are incorporated herein by reference.

The alkenyl monocarboxylic acids can be prepared by halogenating a polymer of a  $C_2$  to  $C_5$  mono-olefin such as polyethylene, polypropylene, or polyisobutylene, with sufficient halogen such as chlorine to provide one to two atoms of halogen per molecule of the olefin polymer, after which the halogenated polymer thus obtained is condensed with an alpha, beta-unsaturated aliphatic monocarboxylic acid of from three to eight carbon atoms, e.g. acrylic acid, crotonic acid, methacrylic acid, etc. Thus, chlorinated polyisobutylene when reacted with acrylic acid will provide polyisobutetyl propionic acid. This high molecular weight acid is then reacted with an aliphatic polyamine such as tetraethylene pentamine, diethylene triamine, octaethylene nonamine, or the like, to form an amide reaction product. The mole ratio of high molecular weight acid to polyamine can range from about 1:1 to about 5:1. See British Pat. No. 1,075,121.

The sulfurized derivatives, i.e. the foregoing amino condensation products reacted with elemental sulfur, are described in detail in U.S. Pat. No. 3,390,086, and an alternative method of preparing such sulfurized ashless dispersants is shown in U.S. Pat. No. 3,309,316. These patents are incorporated herein by reference. A specific dispersant which is especially useful is polyisobutetyl propionic acid condensed with tetraethylene pentamine or polyisobutetyl succinic anhydride condensed with tetraethylene pentamine. The sulfurization of these materials with elemental sulfur is also disclosed in U.S. Pat. No. 3,390,086.

The reaction conditions under which the monomeric or polymeric olefinically unsaturated aliphatic hydrocarbons are subjected to reaction with elemental sulfur, or with sodium polysulfide, generally involve the maintenance of temperatures between about 200° and about 500° F., preferably between about 300° and 450° F. for a time ranging between about 30 minutes and about 40 hours, preferably for between about 4 and about 12 hours. The relative amounts of sulfur

reacted with the organic compounds may vary considerably but are generally between about 0.2 and about 200 moles of sulfur, preferably between about 1 and about 150 moles of sulfur per mole of olefinically unsaturated compound. This will result in a final product containing a combined sulfur content of between about 1.0 and about 10.0 wt. percent sulfur, preferably between about 1.5 and 7.5 wt. percent sulfur. Also the reaction may be carried out using reactants and reaction conditions shown in U.S. Pat. No. 3,390,086.

10 The product may also be prepared using a mineral lubricating oil as a reaction medium solvent or base in which the sulfurization reaction is carried out, in which case the final product constitutes a concentrate of the sulfurized olefinically unsaturated aliphatic hydrocarbon of between about 50 and about 80 percent concentration of the sulfurized compound in the base oil.

15 This is especially useful where the reactant to be sulfurized is normally solid but is oil-soluble also. The ashless dispersant may be added as an oil concentrate in the lubricating oil as a base oil concentrate of 50-70 percent active ingredient concentration.

20 The amount of the sulfurized olefinically unsaturated aliphatic hydrocarbon which is ultimately contained in the final compounded oil, is sufficient, as a minimum, to act as an antioxidant or oxidation inhibitor and at the same time, if the unsulfurized compound possesses viscosity index improving properties, is generally sufficient, in amount, to serve also as a conventional viscosity index improver. Generally this amount 25 will range between about 0.05 and about 10.0 wt. percent based on the oil composition, preferably between about 0.1 and about 5.0 wt. percent, on the same basis. The ashless dispersant, and, optionally, sulfurized ashless dispersant likewise should be present in sufficient amount to impart to 30 the final oil composition recognized beneficial sludge dispersing properties. This generally also amounts to between about 0.05 and about 10.0 wt. percent, preferably between about 0.1 and about 5.0 wt. percent, on the same basis as before stated.

35 40 The lubricating oils are preferably mineral lubricating oil fractions which are derived from naphthenic, paraffinic, aromatic, or mixed crude oils and which are customarily employed as automotive crankcase, diesel engine, gas engine, and heavy duty or railroad diesel engine, oils. Generally, they 45 will have a viscosity at 210° F. of between about 40 and about 90 SUS (Saybolt Universal Seconds) and at 100° F. a viscosity of between about 150 and about 1,000 SUS. The viscosity indices of these oils will generally range between about 0 and about 100 depending upon the specific use to which the oils 50 are to be put. In the case of oils employed in high speed, heavy duty diesel engines, oils of high viscosity indices are often preferred, i.e. of the order of 60-100 or higher, but usually railroad diesel engines employ lubricating oils having viscosities of between about 75 and about 80 SUS at 210° F. and of between about 800 and about 1,250 SUS at 100° F. with viscosity indices ranging between about 55 and about 80.

55 The final compounded lubricating oil compositions may also contain other conventional additives, in addition to the sulfurized viscosity index improvers, each in association with the ashless dispersant and, optionally, with the sulfurized ashless dispersants. These are conventional additives and they 60 are designed to complement and supplement the properties in the final oil which are attainable through the use of the two types of additives herein described and which, in combined use, show the unexpected high temperature properties. Amounts similar to the amounts specified for the novel additives are likewise employed for the conventional additives such as corrosion inhibitors, (sorbitan monooleate), antioxidants, (N-phenyl alpha naphthylamine), pour point depressants, (unsulfurized wax alkylated naphthalene), viscosity index improvers (unsulfurized polyisobutylene or various polymethyl methacrylates, antiwear agents (the zinc salt of di( $C_4-C_8$  alkyl)dithiophosphate), detergents (the alkaline earth metal salts of alkyl substituted phenol thioethers or sul-

fides), and dispersants (alkaline earth metal salts of petroleum sulfonic acids or of alkaryl sulfonic acids) and the like.

A number of routine tests were carried out on compounded oils containing the novel additives hereinbefore described on a comparative basis in order to illustrate the beneficial effect of the combined additives. These tests may be described as follows.

The additive compositions prepared in accordance with the following examples were placed into various mineral lubricating oil bases and were subjected to several types of tests in order to determine their stability at high temperature, as well as under conventional conditions, to inhibit the formation of sludge, to determine their oxidation stability ability, their ability to disperse sludge once it is formed and in general to determine their ability to withstand severe oxidative high temperature conditions. Several tests include a determination of their bearing corrosiveness as well. One or more of the following tests were employed.

1. The Sludge Inhibition Bench Test was employed. This involved the use of a sludge-containing used oil which was rendered free of solid sludge by centrifuging for one hour at 1,800 rpm. The supernatant oil was decanted from the insoluble sludge particles but the oil which was had been freed of solid sludge particles did contain oil-soluble sludge precursors which upon heating as applied in the test would tend to form additional oil-insoluble deposits of sludge. In a tared stainless steel centrifuging tube, 10 grams of supernatant used oil containing from 0.5 wt. percent to 5.0 wt. percent active ingredient to be tested was heated to 300° F. for 2 hours in a constant temperature oil bath. Following the heating, the tube was cooled and then centrifuged for one hour at 1,800 rpm. The supernatant oil was decanted again from the tube and any residual deposits of sludge were washed carefully with 99 percent n-pentane to remove all remaining oil. The weight of the solid sludge formed in the test was determined. A blank or comparative run was also run in which no additive was employed in the oil. A substantial decrease in the amount of sludge deposited as compared with the amount deposited in the case of the blank run indicates that the additive had a sludge inhibiting effect. In addition to an actual measurement, in milligrams, of the weight of the sludge so collected, a haze determination was carried out on the centrifuged supernatant oil. This is done by means of a nephelometer light diffraction reading. The lower the number obtained, the less haze because of the lesser number of particles present to scatter the light.

2. Another test employed in the case of some of the comparative runs is known as the Cyclic Temperature Sludge Test. It was carried out for a total number of hours, depending upon the particular test run, for a minimum of 105 hours and in some cases for a maximum of 168 hours. In order to evaluate the sludge handling ability of the additives in lubricating oil in this test, a Ford 6-cylinder engine was used which employed a standard carburetor. It was operated at a standard speed of 1,500 rpm  $\pm$  15 rpm under a constant load of 140  $\pm$  2 foot-pounds of torque. In this test, the temperature of the oil in the crankcase was cyclically and sequentially raised and lowered during the period of total hours of running the test. The cold phase operation, i.e. the lower temperature, was maintained for a period of 5 hours, alternated with a hot phase operation in which the high temperature was maintained for 2 hours. The oil sump temperature in the cold phase was 150° F.  $\pm$  5° F. and the hot phase operation was 215° F.  $\pm$  5° F. This test was used to determine the oxidation stability and the sludge inhibiting and sludge dispersing tendencies of the novel additive or additives. The base oil employed in this test was free of other additives and would completely breakdown so much so that it was not possible to complete the 240 hours of the run. Even after 100 hours, the top groove fill was excessive and the P.M.-1 rating indicated an extremely dirty piston when using the base oil alone. Using the base oil alone, the test was not, and could not be, continued beyond 100 hours.

3. P In securing some of the following data a test known as the Falex Wear Test was employed. This involves the use of a conventional Falex Wear Test Machine which was operated with the test oils for 30 minutes over 500 pounds per square

5 inch direct pressure, gauge, on a bearing having a rotating steel pin, which bearing was submerged in the test oil. At the end of this time, the steel pin used in the test was weighed in order to determine the amount of wear on the pin in milligrams of lost weight. This test was conducted for the purpose of measuring the amount of wear which the bearings would encounter under extremely severe conditions when operating in a bath of the test oil composition. Pin seizure or borderline pin seizure conditions are avoided, if possible, but if they do occur, the test oil is deemed to have failed in antiwear qualities.

10 4. Still a further type of test was employed in some instances in securing the data hereinafter presented. It is known as a CRC-L-38 Oil Oxidation Test and is designed to determine the bearing weight loss in milligrams obtained in operating conventional standard single cylinder CLR spark ignition engines. Using the test oil, the engine was run for 40 hours at a relatively high speed, i.e. 3,150 rpm at an oil temperature of about 190°-200° F., with the oil sump temperature being somewhere between 275° and 290° F. and at high load. This test determines, inter alia, the oxidative characteristics of the oil, the copper-lead bearing weight loss, and the corrosion which the bearings undergo using the test oil.

15 5. Still a further test involved in securing some of the following data is known as the gas engine detergency and cleanliness test. This involves the testing of compounded lubricating oils, under comparative conditions, in a Chevrolet gas engine of 6 cylinders and of 216.5 cubic inch displacement operating on natural gas and having a horsepower rating of 34 at 1,500 rpm.

20 35 The engine operated at 2.5 percent excess oxygen in the exhaust in order to maximize nitrogen fixation and oil degradation. The test was conducted for a period of 96 hours using a paraffinic base oil containing no additives other than those specified in the following data. This amounted to an SAE 30-grade oil and had an overall viscosity at 100° F. of 540 SUS and at 210° F. of 66 SUS. The paraffinic base stock comprised 90 percent of a solvent neutral 450 SUS at 100° F. and 10 percent of a brightstock of similar characteristic with a viscosity of 150-160 SUS at 210° F. After running for a period of 96 hours, the piston and cylinder, valves, compression grooves, rings and piston undersides were inspected for varnish and sludge and the bearings sometimes were inspected for bearing weight loss, in milligrams. An overall demerit system was employed for inspection and the rating of the various portions of the engines was used in getting the overall merit rating. Zero rating represents a perfectly clean engine and an engine with a 10 rating represents the dirtiest sludge and varnish deposits that it is possible to obtain.

25 40 50 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 95

### EXAMPLE 1

A mixture of 2,490 grams of polyisobutylene having a number average molecular weight of about 900 was reacted with 480 grams of elemental sulfur at a temperature of about 400° F. for 24 hours and was thereafter filtered through a filter aid. The resulting product contained about 8.71 wt. percent of sulfur.

**EXAMPLE 2**

A mixture of 830 grams of the same polyisobutylene as used in Example 1 together with 160 grams of elemental sulfur was heated at 250° F. for 24 hours and filtered through a filter aid. The filtrate contained 2.69 wt. percent of sulfur in chemically combined form.

### EXAMPLE 3

A mixture of 89.7 wt. percent of polyisobutylene of approximately the same molecular weight as that described in the preceding examples and approximately 10.3 wt. percent of elemental sulfur was heated at 400° F. for 12 hours and filtered. The filtrate product showed an analysis of chemically combined sulfur of about 5.2 wt. percent sulfur.

#### EXAMPLE 4

The same mixture as employed in Example 3 was heated at the same temperature as in Example 3 for about 20 hours and filtered through a filter aid. This showed a combined sulfur analysis of about 5.4 wt. percent.

Sulfurized products of the foregoing examples were incorporated into a heavy duty base lubricating oil commonly used in gas engines in varying amounts with and without the addition of conventional ashless dispersants and the compounded oil composition was subjected to various automotive lubrication tests, including test (5) previously mentioned, the results of which are set forth in Table I.

The base oil employed in securing the data shown in Table I was the oil blend (SAE-30 grade), previously described, which comprised 90 percent of solvent neutral paraffinic base stock having a viscosity of 450 SUS at 100° F. and 66 SUS at 210° F. plus 10 percent of a solvent neutral brightstock 150-160 SUS at 210° F.

TABLE I

| Run<br>No. | Additive        | Additive,<br>wt.<br>percent | Lube<br>stability <sup>6</sup><br>test, per-<br>cent vis. |                         | Cu-Pb<br>bearing <sup>6</sup><br>wt. loss,<br>mgs. | L-38 <sup>4</sup><br>bearing<br>wt. loss,<br>mgs. | Gas<br>engine <sup>5</sup><br>overall<br>demerit |
|------------|-----------------|-----------------------------|-----------------------------------------------------------|-------------------------|----------------------------------------------------|---------------------------------------------------|--------------------------------------------------|
|            |                 |                             | increase at<br>100° F.                                    | test, per-<br>cent vis. |                                                    |                                                   |                                                  |
| 1          | None (base oil) | None                        |                                                           | 51                      | -285                                               | >1,000                                            | 0.63                                             |
| 2          | Example 1       | 5                           |                                                           | 17.7                    | +17                                                | 16                                                | 0.36                                             |
| 3          | Example 1       | 3 }                         |                                                           | 15.0                    | +2                                                 | 109                                               | 0.06                                             |
| 4          | (PIBA-TEPA*)    | 2 }                         |                                                           |                         |                                                    |                                                   |                                                  |
| 4          | Example 2       | 5                           |                                                           | 16.7                    | +18                                                |                                                   |                                                  |
| 5          | Example 3       | 4 }                         |                                                           |                         |                                                    |                                                   |                                                  |
| 5          | (PIBA-TEPA)     | 3 }                         |                                                           | 18.0                    | -69                                                | 54                                                | 0.08                                             |
| 6          | Example 4       | 4 }                         |                                                           |                         |                                                    |                                                   |                                                  |
| 6          | (PIBA-TEPA)     | 3 }                         |                                                           | 14.8                    | -1                                                 | 104                                               | 0.11                                             |

\*PIBA-TEPA as used in the foregoing table is the conventional amide condensation product of about 2.8 moles of polyisobutylene propionic acid with each mole of tetraethylene pentamine.

### EXAMPLE 5

About 2,000 grams of polyisobutylene having a number average molecular weight of about 130,000, as a 20 percent concentration in a solvent neutral 150 base lubricating oil, was heated with 20 grams of elemental sulfur at a temperature of about 300° F. for 8 hours. The final product had a sulfur content of 1.08 wt. percent based on the weight of the polyisobutylene.

A base oil blend was prepared in the weight ratio of 9 parts of solvent neutral lubricating oil stock of 100 SUS at 100° F. viscosity which was admixed with each part of solvent neutral 450 SUS at 100° F. viscosity lubricating oil stock. This blend also contained about 1.2 percent of the zinc salt of di(C<sub>4</sub>-C<sub>5</sub> alkyl)dithiophosphate, as an antiwear additive, and lesser but

effective amounts of a commercially available overbased calcium alkaryl sulfonate and of a commercially available pour point depressant which was a 75-25 percent mixture of wax alkylated naphthalene and dilorol fumarate-vinyl acetate copolymer.

Cyclic Temperature Sludge Tests (2) were carried out as a series of comparative runs with all runs employing the above described base oil compounded as therein described. The test results were as follows:

TABLE II

| Run No. | Additive, Wt. %                                                                                             | Hours 63 | 105  | 147 | 168 |
|---------|-------------------------------------------------------------------------------------------------------------|----------|------|-----|-----|
| 7       | 10.6 wt. % sulfurized polyisobutylene                                                                       |          | 5.4  |     |     |
| 8       | 10.6 wt. % unsulfurized polyisobutylene plus 3.8 wt. % PIBSA/TEPA                                           | 9.23     | 5.5  |     |     |
| 9       | 10.6 wt. % sulfurized polyisobutylene plus 3.8 wt. % PIBSA/TEPA                                             | 9.94     | 9.45 | 6.8 | 5.6 |
| 10      | 1.0 wt. % sulfurized polyisobutylene plus 10.0 wt. % unsulfurized polyisobutylene plus 3.8 wt. % PIBSA/TEPA | 9.94     | 9.38 | 5.9 |     |

\*PIBSA/TEPA is the conventional amide condensation ashless dispersant produced in accordance with the teachings of U.S. Pat. No. 3,172,892.

The numbers in the foregoing Table give sludge ratings wherein 10 represents a perfectly clean engine and 0 represents the worst possible dirty engine. From these data, it is obvious that a beneficial synergistic sludge inhibition effect is achieved through the combined use of sulfurized polyisobutylene and a conventional ashless dispersant (Run 9).

40 A base oil blend was prepared of the same two lube oil stocks in the same weight ratios. The same additives, in the same amounts, were added to the blended base except that the dithiophosphate antiwear agent was omitted and 3.8 wt. per-

Comparative Falex Antiwear Tests (3) were carried out using this compound, the results being:

65 using this compounded base oil at 500 lbs. per square inch pressure for 30 minutes. The following data were obtained:

TABLE III

| Run No. | (Mgs.) Bearing Weight Loss                    |
|---------|-----------------------------------------------|
| 11      | Base oil + 10.6% unsulfurized polyisobutylene |
| 12      | Same as Run 11 + 1.2% zinc                    |

|    |                                                                                                                         |            |
|----|-------------------------------------------------------------------------------------------------------------------------|------------|
| 13 | di (C <sub>4</sub> -C <sub>8</sub> alkyl) dithiophosphate<br>Base oil + 10.6% sulfurized<br>polyisobutylene (Example 5) | 5.5<br>7.0 |
|----|-------------------------------------------------------------------------------------------------------------------------|------------|

These data indicate that the product of Example 5 also exhibits substantial antiwear activity (Run 13) as an additional desired property even though it does not appear to have superior qualities in this regard when compared to the use of conventional commercially available antiwear agents (Run 12).

The sulfurized polyisobutylene of Example 5 was further comparatively tested in the Sludge Inhibition Test (1) wherein a used lubricating oil containing sludge precursors but free of suspended sludge was employed to determine the sludge inhibiting properties of the compound. The following test results were obtained:

TABLE IV

| Run No. |                                                            | Mgs. of Sludge<br>Per 10 Grams<br>Used Oil |
|---------|------------------------------------------------------------|--------------------------------------------|
| 14      | Used Oil                                                   | 12.0                                       |
| 15      | 0.4 wt. % PIBSA.TEPA.HAc*                                  | 3.5                                        |
| 16      | + Used Oil                                                 | 3.4                                        |
| 17      | Same as Run 15 + 1% polyisobutylene                        | 1.5                                        |
|         | Same as Run 15 + 1% sulfurized polyisobutylene (Example 5) |                                            |

\*Prepared according to U.S. Patent 3,172,892.

These data illustrate the sludge inhibiting synergism in using the combination of an ashless dispersant (PIBSA.TEPA. HAc) with sulfurized polyisobutylene (Run 17) in contrast to the use of the dispersant alone (Run 15) or the unsulfurized polyisobutylene (Run 16) of Example 5.

## EXAMPLE 6

About 200 grams of ethylene/propylene copolymer having a number average molecular weight of about 100,000 was treated in a light lubricating oil serving as a solvent, with about 8 grams of elemental sulfur at a temperature of about 356° F. for 9 hours. After filtration to remove any unreacted sulfur the filtrate was found to contain 2.87 wt. percent of combined sulfur based upon the ethylene/propylene copolymer starting reactant.

Used lubricating oil containing sludge precursors but being free of undissolved sludge was subjected to the sludge inhibition test (1) under comparative conditions, in which 1 percent of the starting unsulfurized ethylene/propylene copolymer was used in one instance and 1 percent of the sulfurized ethylene/propylene copolymer was used in the other instance. The unsulfurized copolymer was found to have produced 20.1 milligrams of sludge per 10 grams of used oil while the sulfurized copolymer produced 20.3 milligrams of sludge on the same basis. However, the same two tests were repeated using the same amount of sulfurized and unsulfurized copolymer but in each case with 0.4 wt. percent of conventional ashless dispersant being present, namely the amide condensation product of polyisobutylene succinic anhydride with tetraethylenepentamine. The sulfurized copolymer, in that combination, showed only 1.7 milligrams of sludge during the sludge inhibition test whereas the unsulfurized copolymer, in such combination, showed 3.2 milligrams of sludge. On a comparative basis, the same oil containing 0.4 wt. percent of the ashless dispersant but no copolymer additive, of either type, showed a final solid sludge formation of 3.5 milligrams per 10 grams of used oil.

## EXAMPLE 7

A mixture of C<sub>20</sub><sup>+</sup> alpha monoolefins in the amount of about 200 grams was reacted with about 10 grams of sulfur at a temperature of about 176° F. for 12 hours. The final product contained about 4.61 wt. percent of combined sulfur. This material was subjected to the same sludge inhibition test (1) as the product of Example 6 employing a used lubricating oil, and the same comparative tests were run including the comparative test using the conventional ashless dispersant alone described in Example 6. The results were as follows:

TABLE V

|                                                                                                   | Sludge, Milligrams<br>Per 10 Grams Used<br>Oil |
|---------------------------------------------------------------------------------------------------|------------------------------------------------|
| 1% C <sub>20</sub> <sup>+</sup> alpha olefins (sulfurized)                                        | 15.4                                           |
| 1% C <sub>20</sub> <sup>+</sup> alpha olefins (unsulfurized)                                      | 15.1                                           |
| 1% C <sub>20</sub> <sup>+</sup> alpha olefins (sulfurized) plus<br>0.4 wt. % ashless dispersant*  | 7.0                                            |
| 1% C <sub>20</sub> <sup>+</sup> alpha olefins (unsulfurized)<br>plus 0.4 wt. % ashless dispersant | 10.1                                           |
| 0.4 wt. % ashless dispersant (alone)                                                              | 9.8                                            |

\*Same dispersant as used in Example 6.

## EXAMPLE 8

A polyisobutylene of about 300 number average molecular weight in the amount of 300 grams was reacted with 32 grams of elemental sulfur at a temperature of about 355° F. for 8 hours. After stripping the product with nitrogen gas for 1 hour, the product was found to contain about 5.2 wt. percent of combined sulfur.

The same used oil was employed in the sludge inhibition test (1). The product of Example 8 was added to the used oil and the sludge inhibition test carried out. On the same comparative basis as described in the two preceding examples, the following results were obtained:

TABLE VI

|                                                                                                              | Sludge, Milligrams<br>Per 10 Grams Used<br>Oil |
|--------------------------------------------------------------------------------------------------------------|------------------------------------------------|
| 1% sulfurized polyisobutylene<br>of Example 8                                                                | 9.4                                            |
| 1% unsulfurized polyisobutylene<br>(reactant of Example 8)                                                   | 11.3                                           |
| 1% sulfurized polyisobutylene plus 0.4 wt. %<br>conventional ashless dispersant as described<br>in Example 6 | 1.4                                            |
| 1% unsulfurized polyisobutylene plus 0.4 wt.<br>% ashless dispersant                                         | 2.7                                            |
| 0.4 wt. % ashless dispersant (alone)                                                                         | 2.8                                            |

## EXAMPLE 9

Polyisobutylene having a number average molecular weight of about 900, in the amount of 500 grams, was reacted with 50 grams of elemental sulfur at a temperature of about 482° F. for about 6 hours. After stripping the reacted mixture for about 1 hour under nitrogen gas, the product was analyzed and found to contain 3.15 percent of combined sulfur.

Used lubricating oil containing sludge precursors was used as the base test oil for a comparative series of sludge inhibition tests (1) as previously described which gave the following results:

TABLE VII

|    | Sludge, Milligrams |
|----|--------------------|
| 75 |                    |

|                                                                                   | Per 10 Grams Used |
|-----------------------------------------------------------------------------------|-------------------|
| Oil                                                                               |                   |
| 1 wt. % polyisobutylene (reactant of Example 9)                                   | 11.3              |
| 1 wt. % sulfurized polyisobutylene (Example 9 product)                            | 11.3              |
| 2 wt. % unsulfurized polyisobutylene plus 0.4 wt. % ashless dispersant*           | 4.5               |
| 2 wt. % sulfurized polyisobutylene plus 0.4 wt. % conventional ashless dispersant | 0.7               |
| 0.4 wt. % ashless dispersant (alone)                                              | 3.4               |

\*Same dispersant as used in Examples 6-8.

From the above examples it is apparent that the combination of sulfurized olefinically unsaturated hydrocarbons and conventional ashless dispersants has a synergistic effect on the inhibition of oxidation inhibition of sludge formation, and a corrosion and wear protection of sensitive bearing materials.

The Lube Stability Test (5) data illustrate the effectiveness of the sulfurized materials as oxidation inhibitors and in reducing Cu-Pb bearing corrosion. The presence of ashless dispersants does not change this effectiveness (by itself the dispersant would provide no such protection), while the combination of the two types of additives provides a degree of engine cleanliness (gas engine test 5) that cannot be achieved by either alone.

The L-38 Test (4) data show that the sulfurized materials provide Cu-Pb bearing protection.

The Cyclic Temperature Sludge Test (2) demonstrates the ability of the combined additives to provide less sludge and varnish than can be obtained by either one alone. Results from this test correlate with passenger car engine performance. Reduction of wear in the Falex Test (3) is important because of its relationship to passenger car engine wear.

The Bench Sludge Inhibition Test (1) shows synergism and is important because its results correlate with the Cyclic Temperature Sludge Test (2).

What is desired to be secured by Letters Patent follows.

I claim:

1. A lubricating oil composition comprising a major proportion of a mineral lubricating oil, a minor sludge inhibiting amount of at least one oil-soluble sulfurized hydrocarbon produced by sulfurizing an oil-soluble olefinically unsaturated hydrocarbon having a number average molecular weight between about 200 and about 150,000 and selected from the group consisting of monomeric alpha monoolefins of at least 16 carbon atoms per molecule; homopolymers of  $C_2-C_{18}$  alpha monoolefins; copolymers of  $C_2-C_{18}$  alpha monoolefin with a different  $C_3-C_{18}$  alpha monoolefin; and terpolymers of a  $C_2-C_{18}$  alpha monoolefin, a different  $C_3-C_{18}$

alpha monoolefin and a third monomer which is either a third and still different  $C_3-C_{18}$  alpha monoolefin or a  $C_4-C_{18}$  diolefin, and a minor sludge dispersing amount of at least one oil-soluble ashless sludge dispersant selected from the group consisting of condensation products of aliphatic polyamines with long chain alkenyl aliphatic monocarboxylic acids, dicarboxylic acids and dicarboxylic acid anhydrides wherein the alkenyl radical has from about 40 to 250 carbon atoms.

2. A lubricating oil composition as in claim 1 wherein the amount of sulfurized hydrocarbon and the amount of ashless sludge dispersant are each between about 0.05 and about 10.0 wt. percent of the total oil composition.

15 3. A lubricating oil composition as in claim 1 wherein the hydrocarbon subjected to sulfurization is at least one  $C_{16}^+$  monomeric alpha monoolefin.

4. A lubricating oil composition as in claim 3 wherein the hydrocarbon subjected to sulfurization is a mixture of  $C_{20}^+$  monoolefin monomers.

5. A lubricating oil composition as in claim 1 wherein the hydrocarbon subjected to sulfurization is at least one homopolymer of a  $C_2-C_{18}$  alpha monoolefin.

6. A lubricating oil composition as in claim 5 wherein the hydrocarbon subjected to sulfurization is a polyisobutylene.

7. A lubricating oil composition as in claim 1 wherein the hydrocarbon subjected to sulfurization is at least one copolymer of a  $C_2-C_{18}$  alpha monoolefin with a different  $C_3-C_{18}$  alpha monoolefin.

30 8. A lubricating oil composition as in claim 7 wherein the hydrocarbon subjected to sulfurization is a copolymer of ethylene and propylene.

9. A lubricating oil composition as in claim 1 wherein the hydrocarbon subjected to sulfurization is at least one terpolymer of a  $C_2-C_{18}$  alpha monoolefin, a different  $C_3-C_{18}$  alpha monoolefin and a third monomer which is either a third and still different  $C_3-C_{18}$  alpha monoolefin or a  $C_4-C_{18}$  diolefin.

10. A lubricating oil composition as in claim 1 which also 40 contains a minor sludge inhibiting amount of at least one sulfurized ashless dispersant wherein said ashless dispersant is as set forth in claim 4.

11. A lubricating oil composition as in claim 1 wherein the alkenyl radical is derived from polyisobutylene.

45 12. A lubricating oil composition as in claim 1 wherein said condensation product is obtained from tetraethylene pentamine and polyisobutylene succinic anhydride.

13. A lubricating oil composition as in claim 1 wherein said condensation product is obtained from tetraethylene pentamine and polyisobutylene propionic acid.

\* \* \* \* \*